

# United States Patent [19]

Zabolotsky et al.

[11] 3,811,166

[45] May 21, 1974

[54] **METHOD OF MAKING SPLIT METAL PACKING RINGS**

[76] Inventors: **Grigory Mikhailovich Zabolotsky, Karamyshevksya naberezhnaya, 24, kv. 27; Vladimir Mikhailovich Rakovsky, Ulitsa petrozavodskaya, 15, Korpus 1, kv. 65, both of Moscow; Sergei Alexandrovich Shuster, Krasnogorodsky raion, poselok Opalkha, ulitsa Leninskaya, 13, kv. 5, Moskovskaya Oblast; Mikhail Vsevolodovich Boldyrev, Ulitsa putevoi proezd, 38, kv. 77, Moscow, all of U.S.S.R.**

[22] Filed: Nov. 3, 1971

[21] Appl. No.: 195,190

[52] U.S. Cl. .... 29/156.6

[51] Int. Cl. .... B23p 15/06

[58] Field of Search .... 29/156.6; 72/340; 277/216, 277/217, 225

[56] **References Cited**

UNITED STATES PATENTS

2,591,920 4/1952 Colvin..... 277/216

|           |         |               |          |
|-----------|---------|---------------|----------|
| 2,212,336 | 8/1940  | Wenzel .....  | 277/216  |
| 3,414,277 | 12/1968 | Schmidt ..... | 277/216  |
| 929,484   | 7/1909  | Petter .....  | 29/156.6 |
| 3,561,087 | 2/1971  | Koehler ..... | 29/156.6 |
| 2,362,810 | 11/1944 | Farr .....    | 277/216  |

Primary Examiner—Charles W. Lanham

Assistant Examiner—M. J. Keenan

Attorney, Agent, or Firm—Holman & Stern

[57]

## ABSTRACT

A circular ring blank is strained to impart radial springiness or resiliency thereto by way of a reduction (compression) of the opposite outer flat surfaces thereof on the sections adjacent to the cylindrical surface opposite to its cylindrical sealing surface. Maximum reduction force is applied to the outer flat surfaces that lie against the split and as far as half the width of the ring width, with the same being gradually decreased to zero on the outer flat surfaces adjacent to the ring split.

2 Claims, 15 Drawing Figures





FIG. 2



FIG. 1



FIG. 6



FIG. 3



FIG. 7



FIG. 5



FIG. 8



FIG. 10



FIG. 9



FIG. 11



FIG. 12



FIG. 13



FIG. 14



FIG. 15

## METHOD OF MAKING SPLIT METAL PACKING RINGS

### BACKGROUND OF THE INVENTION

The present invention relates generally to plastic metal working practice and more specifically, to a method of making split metal packing rings.

The present method is instrumental in making packing rings, in which sealing surfaces are in fact the outside cylindrical surface and face surfaces (the so-called outside-pressure rings, i.e., piston rings), as well as packing rings, in which the sealing surfaces are, in effect, the inside cylindrical surface and face surfaces. Unlike pistons these will hereinafter be referred to as inside-pressure rings.

### PRIOR ART

All the heretofore-known methods of making split metal packing rings differ in the principle underlying the ring-shaping process, i.e., the rings, when free, have imparted thereto such an out-of-round shape that when fitted into a cylinder (in case of packing rings) or fitted onto the piston rod or a sphere (in case of inside-pressure rings), they would have a circular shape and exert largely a uniform pressure upon the adjacent surface of the part being packed (cylinder or piston rod) throughout its periphery.

Known in the art is a method of making split metal inside-pressure packing rings, in which a circular turned ring blank has imparted thereto the desired elastic properties to suit the requirement of exerting a uniform inside pressure by the ring when in its working position, due to straining said ring blank in a radial direction by radial indents or notches made on the outside cylindrical surface of the ring blank with a preset-shaped driftpin. The indents or notches result from strikes delivered against the outside cylindrical surface of the ring blank at the same force but spaced apart from one another circumferentially at an ever-increasing distance (at variable pitch) so that the minimum notch spacing is given to the surface lying against the ring split and the maximum spacing, to the surface adjacent to the split. Notches can be made on the outside cylindrical surface of the ring blank at a regular pitch as well, but by gradually increasing the striking force and, consequently, the notching depth so that the maximum force is applied to the ring surface located against the split and the minimum force, to that adjacent to the ring split.

A disadvantage inherent in said method is that it is highly laborious and, consequently, a low-efficiency method since 120 to 180 notches of different depths or pitches are to be made on the outside cylindrical surface of a ring blank in order to strain it by the above mentioned method.

Besides, there is known to be in widespread use, a method of making piston rings, in which the required out-of-round shape of the ring when in free state is obtained by casting a non-round ring blank followed by a mechanical treatment of said blank to a former or templet.

The method, however, suffers likewise from complexity and high labor consumption of the production process, since it requires an individual casting of every ring blank and subsequent milling of a variable-curvature ring to a former or templet.

### OBJECTS AND SUMMARY OF THE INVENTION

It is an object of the present invention to provide a simpler and less laborious method of making packing rings.

It is another object of the present invention to provide a method of making packing rings which is highly efficient.

According to the above and other objects, provision is made for a method of making packing rings, in which a circular ring blank is strained to impart radial elastic properties (springiness) thereto, whereupon said ring is subject to a consecutive machining on the face, the outside cylindrical and inside cylindrical surfaces thereof, and in which, according to the invention the ring blank is strained by reduction of the opposite outer flat surfaces thereof on the sections adjacent to its outside cylindrical surface lying opposite to the ring cylindrical sealing surface; maximum reduction force is applied to the outer flat surfaces lying against the split of the ring blank as far as half the width of the ring and is gradually decreased to a minimum when applied to the outer flat surfaces close to the split of the ring blank.

It is expedient, when making packing rings, in which the outside cylindrical surface serves as a sealing surface, to reduce the sections of the opposite outer flat surfaces of the ring blank which are adjacent to the inside cylindrical surface thereof.

Reduction of such a section of the outer flat surface of the ring blank is used when making piston rings.

It is likewise practicable, when making packing rings, in which the inside cylindrical surface serves as a sealing surface, to reduce the sections of the ring blank end faces which are adjacent to the outside cylindrical surface thereof.

Reduction of such a section of the outer flat surface of the ring blank is used when making inside-pressure rings.

The present method of making split metal packing rings, though simple and non-laborious, renders high production capacity and good quality of the packing rings produced.

Given below is a description of specific embodiments of the present invention with due reference to the accompanying drawings, wherein:

### BRIEF DESCRIPTION OF THE DRAWING

FIG. 1 shows an inside-pressure packing ring while in a working position;

FIG. 2 is a view partly in elevation and partly in cross section of a reducing die with plane working surfaces which embodies a method of making split inside-pressure packing rings, according to the invention and a ring blank placed therein;

FIG. 3 is a view taken along line III—III in FIG. 1, the view looking in the direction of the arrows;

FIG. 4 is a side view of an inside-pressure packing ring while in an inoperative position;

FIG. 5 shows a piston ring while in a working position;

FIG. 6 is a fragmentary view partly in elevation and partly in cross section of a reducing die with plane working surfaces which embodies a method of making piston rings, according to the invention and a ring blank placed therein;

FIG. 7 is a view taken along line VII—VII in FIG. 5, the view looking in the direction of the arrows;

FIG. 8 is a side view of a piston ring while in an inoperative position;

FIG. 9 is a fragmentary view partly in elevation and partly in cross section of a reducing die having a punch with an inner taper working surface, to embody a method of making inside-pressure packing rings, according to the invention and a ring blank placed therein;

FIG. 10 is a view taken along line X—X in FIG. 1, the view looking in the direction of the arrows;

FIG. 11 is a fragmentary view partly in elevation and partly in cross section of a reducing die, wherein its punch has an outer taper working surface, to embody a method of making piston rings, and a ring blank placed therein;

FIG. 12 is a fragmentary view partly in elevation and partly in cross section of a reducing die, wherein its punch features an inner planotaper working surface to make inside-pressure rings;

FIG. 13 is a view illustrating an inner-pressure ring reduced in the die, while in a working position;

FIG. 14 is a fragmentary view partly in elevation and partly in cross section of a reducing die, wherein its punch features an outer planotaper working surface to make piston rings; and

FIG. 15 is a view illustrating a piston ring reduced in the die, while in working position.

#### DETAILED DESCRIPTION OF THE INVENTION

Now referring to the drawings, the method of making inside-pressure packing rings 1 (FIG. 1), in which the inside cylindrical surface of a diameter  $d$  serves as a sealing surface, resides in that to impart to the packing ring a radial springiness and a uniform inside pressure, a preliminarily heat-treated circular ring blank 2 (FIG. 2), is placed in a die 3 whose punch 4 and bottom block 5 have plane working surfaces, in such a manner that the working surfaces of the bottom block 5 and the punch 4 reduce those sections 6 (FIG. 1) of the opposite outer flat surfaces which lie between the circumference of a mean diameter  $= d+t$  and the circumference of an outside diameter  $D$  (i.e., outside cylindrical surface). In FIG. 1, section 6 being reduced of one outer flat surface is shown crosshatched. For the sake of clarity, in the specification only one section will be under consideration but it should be borne in mind that all discussed herein holds equally true of the same section lying on the opposite outer flat surface of the ring blank. Height  $h$  of the section 6 being reduced is a variable quantity, viz., its maximum value  $h_{max}$  = should not be more than  $t/2$  and is located on the outer flat surface of the ring 1 lying against the split, whereupon said quantity gradually decreases to a minimum value ( $h_{min}=0$ ) effective on the outer flat surface close to the split.

Then, the blank 2 is reduced by the pressing effort transmitted to the punch 4 through a spherical support 7, the amount  $a$  (FIG. 3) of the ring strain by its thickness  $b$  a constant quantity.

In this case, a uniform inside pressure exerted by the packing rings 1 while in a working position is ensured due to the fact that the width  $h$  of the section 6 of the ring blank 2 being reduced throughout its length which is determined at any cross-section taken along an arc by an angle  $\phi$ , is of variable character and can be found from the formula:

$$h = b/a \cdot 2/3\pi \cdot A/d+t (1 + \cos \phi) \quad (1)$$

where

$b$  is the thickness of the ring 1;  
 $a$  is the strain value (reduction depth) in thickness  $b$  of the ring 1;  
 $b/a$  is a reciprocal of compressive strain;  
 $d$  is the inside diameter of the ring 1;  
 $t$  is the width of the ring 1;  
 $d+t$  = the ring mean diameter.

10 A is the amount of overlap of the ends of the ring 1 while in a free state (i.e., inoperative) which depends (with the given values of the ring parameters  $d$ ,  $t$  and  $b$ ) upon the preset unit pressure;

15  $\phi$  is an angle (coordinate  $h$ ) taken from the ring midpoint (i.e., the point opposite to the split) towards the split and variable through  $0^\circ$  to  $\pi$  ( $0^\circ$  to  $180^\circ$ ).

The physical meaning of the straining resides in that in the material of the reduced sections 6 of the packing ring there arise extra stresses (as compared to non-reduced sections 8) variable lengthwise of the branches of the ring 1. (By the branch of the rings 1 is meant the length from the point lying against the split to the end adjacent thereto). The extra stresses result in variable radial turns of the ring 1 branches on which account 25 the ring, when free, assumes the preset out-of-round shape and the ends of the branches thereof become overlapped as is shown in FIG. 4.

In an ideal case, i.e., leaving out of account the actual out-of-straight of the die 3 punch guides, the working 30 surfaces of the punch 4 and the bottom block 5 are of plane shape variable only to the width of the section 6 of the ring 1 being reduced and determined by the formula (I). Thus, e.g., with the compressive strain value  $a/b = 1\% = 1/100$  (selected experimentally), the equation (I) for calculating the inside working edges of the punch 4 and the bottom block 5 will be:

$$h = 200/3 \cdot A/d+t(7 + \cos \phi) \quad (II)$$

The above-given curve for inside-pressure rings is in 40 fact a circumference of the diameter  $D_1 = d + 2t - h_{max}$  and is the diameter of the inner border line of the reduced section 6 of the ring 1 outer flat surface and the inside diameter of the edge of the working surfaces of the punch 4 and the bottom block 5. Besides, the center of the circumference is offset with respect to that of the ring 1 along an axis 9 passing through the split of the ring 1, towards said split by an amount of eccentricity equal to

$$e = h_{max}/2$$

45 As a result of a reduction of the section 6 in the die 3, there arise stresses in the material of the ring 1 under which the ring acquires a radial springiness on the side of the inside diameter  $d$ , while due to a variable character of reduction along the ring outside periphery, the ring features a uniform compression diagram on the side of the inside diameter thereof.

Upon having been reduced in the die 3, the ring 1 is subjected to a conventionally known mechanical treatment as follows. The ring 1 is ground on the outer flat surfaces to a preset size, whereupon a number of rings 60 1 in a quantity of 15 to 20 are fitted onto an inside mandrel (not shown), clamped with nuts on the outer flat surfaces and the whole group of the rings is ground along the outside diameter  $D$  to a preset size. When, the inside mandrel together with the rings fitted thereon, is inserted into an outside mandrel, in which the rings 1 are brought into alignment with respect to

the machined outside diameter  $D$ , clamped with the nut of the outside mandrel, whereupon the inside mandrel is removed and the rings 1 are ground along the inside diameter  $d$ . Upon grinding, the inside diameter  $d$  of the ring 1 is lapped to a working size.

To make split metal packing rings 10 (FIG. 5) featuring a uniform outside pressure, i.e., packing rings, in which the outside cylindrical surface serves as a sealing surface (viz., piston rings), a ring blank 11 (FIG. 6) is placed in a die 12 with plane working surfaces to reduce a section 13 of the outer flat surface thereof adjacent to the inside cylindrical surface of diameter  $d_1$ . The width  $h_1$  of the section 13 being reduced, just as in the case of the rings 1, is a variable quantity, viz., its maximum value  $h_{1\ max}$  should not be more than  $t/2$  and is located on the outer flat surface of the ring lying against the split, said quantity  $h_1$  being gradually decreased to a minimum value ( $h_{1\ min} = 0$ ) effective on the outer flat surface close to the split. The quantity  $h_1$  is found from the same formula as the quantity  $h$  for the inside-pressure rings 1, with the sole exception that the quantity  $A$  (denoting the amount of overlap of the ring ends with the ring in free state) is substituted for the quantity  $L$  (FIG. 8) by which the ends of the ring 10 are set apart when in a free state (i.e., while the ring 10 is inoperative), said quantity depending upon the value of the required external pressure.

$$h_1 = b_1/a_1 \cdot 2/3\pi \cdot L/d_1 + t_1 (1 + \cos \phi) \quad (III)$$

The section 13 being reduced of the piston ring 10 is shown crosshatched in FIG. 5.

With a compressive strain equal to  $a_1/b_1 = 1\% = 1/100$ , equation (III) for calculating the outer working edge of a punch 14 and a bottom block 15 of the die 12 will be as follows:

$$h_1 = 200/3\pi \cdot L/d_1 + t_1 (1 + \cos \phi) \quad (IV)$$

For the piston rings 10, this curve is in fact a circumference having the diameter  $D_1 = d_1 + h_{1\ max}$  whose center is offset with respect to the center of the ring 10 along an axis 16 passing through the split of the ring 10 away from said split by an amount of eccentricity equal to

$$e_1 = h_{1\ max}/2$$

Due to such a reduction of the section 13 of the ring 10, stresses arise in the material thereof under which the ring 10 acquires radial elastic properties on the side of the outside diameter  $D_1$ . When in a working position, the ring 10 features a uniform pressure along the outside diameter  $D_1$ .

Upon having been reduced, the ring 10 is subject to a heat treatment (thermal fixing), whereupon the ring undergoes consecutive mechanical treatment on the outer flat surfaces, and the inside and outside cylindrical surfaces thereof to a desired size in a way similar to the inside-pressure rings 1.

Reduction of a circular ring blank 17 (FIG. 9) to obtain an inside-pressure ring may also be made in a die 18, whose punch 19 has an inner working surfaces tapered at an apex angle  $\alpha$ , while the working surface of a bottom block 20 is plane and is square with the cylindrical face of the ring blank 17. The punch 19 and the bottom block 20 are so set that their center is offset relative the center of the ring blank 17 by an amount of eccentricity equal to  $e_2 = h_{2\ max}/2$  towards the ring split as in the case of the inside-pressure ring 1 (FIG. 1).

Width  $h_2$  (FIG. 10) of the section being reduced of the ring blank 17 is a variable quantity, with its maxi-

mum value being on the outer flat surface opposite to the split and the minimum value, close thereto. Besides, the strain value  $a_2$  applied to the ring by the thickness  $b$  when reduction is made in the tapered-surface die 18, is likewise a variable quantity.

Reduction of the outer sections of the ring blank 17 occurs in a radial section and assumes the shape of a triangle having legs  $h_2$  and  $a_2$ ; it follows the following law:

$$10 \quad h_2 a_2 = 4b/3\pi \cdot A/d + t (1 + \cos \phi) \quad (V)$$

Letter symbols in the above formula are the same as in formula (I).

FIG. 11 represents a die 21 for making piston rings. 15 The die has a punch 22 provided with inner working surfaces tapered at a taper apex angle  $\alpha_1$ . The punch 22 and a bottom block 23 are offset with respect to a ring blank 24 by an amount of eccentricity  $e_4$  away from the split.

When calculating a compressive strain of piston rings, use is made of formula (IV) with the sole exception that the overlap quantity  $A$  is substituted for the quantity  $L$  denoting the ring end-to-end distance when the ring is in a free state. As to other particulars, the reduction process is similar to that above described.

It is likewise practicable to effect a reduction of a ring blank 25 (FIG. 12) to obtain an inside-pressure ring 26 (FIG. 13) in a die 27 (FIG. 12), in which the working surfaces of a punch 28 and a bottom block 29, with respect to the outer flat surface of the ring blank 25, have a shape planobevelled towards the split of the ring blank 25 and variable with the thickness thereof by the value  $a_3/2$  of the compressive strain applied thereto. Besides, the maximum value of  $a_3\ max/2$  will occur on that section of the outer flat surface of the ring blank 25 which lies opposite to the ring split, while the value will be decreased to zero close to the split.

The strain value  $a_3$  is found from the formula:

$$a_3 = b/h \cdot 2/3\pi \cdot A/d + t (1 + \cos \phi) \quad (VI)$$

Letter symbols in the above formula as the same as in formula (I).

When reducing the ring blank 25 the reduction width is the same throughout the perimeter of the ring 26.

45 The punch 28 and the bottom block 29 are set concentrically with the ring blank 25, with section 30 being reduced being shown crosshatched in FIG. 13.

Reduction of a ring blank 32 in a die 31 (FIG. 14) having planobevelled working surfaces to obtain a piston ring 33 (FIG. 15) is similar to that above described. The strain value  $a_4$  can be obtained from formula (6), with the sole exception being that the ring end overlap value  $A$  is substituted for the ring end setting apart value  $L$ .

50 Upon having been reduced, the rings 26 and 33 assume a rectangular shape in a radial section.

In all of the above-described variants, the variable character of the ring blank reduction is ensured due to an appropriate shape of the working surfaces of the punch and bottom block. The surfaces should be in a strict agreement with each other circumferentially and of fixed quantity, while the minimum zone of reduction of a ring blank (close to the split) should be marked on the outside of the bottom block with, say, a notch.

With the above-disclosed method of making piston rings whose consumption in the present day technology may amount to billions, an individual casting of every

ring blank and milling variable-curvature rings to a templet are completely eliminated which results in a considerable monetary saving.

A still greater economical effect may be obtained when the present method is used in making inside-pressure packing rings as compared to the conventional method of straining a ring blank by the notching method, since the straining process of a ring blank by the present method occurs in 1-2 steps of reduction in a die and takes a period of time spent approximately for making two notches out of 120-180 required by the known method, i.e., approximately 60-90 times as fast.

What we claim is:

1. A method of making split metal packing rings in which the inside cylindrical surface serves as a sealing surface, comprising the steps of heat treating a circular ring blank for imparting a homogeneous structure to the blank material, subjecting said blank to straining for imparting elastic properties thereto effective in a radial direction, by reduction of the opposite outer flat surfaces thereof on its sections adjacent to the outside cylindrical surface of the blank to a value not greater

than half of the width of the ring blank in the section diametrically opposite to the split of the ring blank and compression is gradually decreased along an arc 180° to a minimum value at the ends of the blank in the place of the split, and consecutively machining the blank on its outer flat surfaces and inside and outside cylindrical surfaces to a preset size.

2. A method of making split metal packing rings in which the outside cylindrical surface serves as a sealing surface, comprising the steps of straining a circular ring blank for imparting radial springiness thereto by reduction of the opposite outer flat surfaces thereof on its sections adjacent to the inside cylindrical surface of the blank to a value not greater than half of the width of the ring blank in the section diametrically opposite to the split of the ring blank and compression is gradually decreased along an arc 180° to a minimum value at the ends of the blank in the place of the split, heat treating the blank for imparting a homogeneous structure to the material thereof and consecutively machining the blank on its outer flat surfaces and inside and outside cylindrical surfaces to a preset size.

\* \* \* \* \*

25

30

35

40

45

50

55

60

65